

## UNITED STATES PATENT OFFICE

LEO P. CHEBOTAR, OF BEACON, NEW YORK, ASSIGNOR TO THE TEXAS COMPANY, OF NEW YORK, N. Y., A CORPORATION OF DELAWARE

## MOTOR FUEL

No Drawing.

Application filed February 27, 1932. Serial No. 595,685.

This invention relates to motor fuels and more particularly to the provision in the fuel of an antioxidant or inhibitor to the effect stabilization against gum formation, 5 change in color, anti-knock property or other alterations which tend to decrease the value thereof.

According to the invention, a motor fuel, such as cracked gasoline or other fuel which 10 tends to undergo alterations as a result of polymerization or autoxidation, is treated by adding thereto the components of an antioxidant and then developing the antioxidant in situ by reacting with said components an 15 oxidizing agent.

It has been customary in stabilizing gasoline with antioxidants heretofore to select a compound which has been previously prepared and then to add the prepared compound 20 to the gasoline that is desired to be stabilized.

Instead of first preparing the antioxidant and then adding it to the gasoline, I have discovered that the antioxidant can be produced in situ by adding predetermined quantities of the components of the desired antioxidant to the gasoline and then reacting these components with the peroxides formed in the gasoline. By this means the 25 antioxidant can be developed as required and much expense and time in preparation thereby avoided. Thus, by adding phenol and para-phenylene-diamine to gasoline there is developed by the peroxides which 30 may be formed in the gasoline indophenol, which has been found to be an effective antioxidant as described and claimed in my co-pending application Serial Number 493,916, filed November 6, 1930.

40 It is well known that motor fuels, such as many cracked gasolines containing unsaturated hydrocarbons, are unstable when exposed to light or air. The cause of this instability has been found to be due largely 45 to formation therein of peroxides which cause formation of undesirable secondary reaction products in the fuel. The peroxides themselves are powerful oxidizing agents and react with oxidizable compounds, 50 themselves thereby becoming reduced.

Therefore, by adding certain oxidizable materials to the motor fuel, oxidation of the materials to the desired extent by the peroxides is readily obtained.

In accordance with my invention, I may 55 add the components of the antioxidant to the gasoline either before or after peroxides are formed. When the gasoline already contains peroxides, the formation of the antioxidant takes place immediately. It is 60 preferred, however, to add the components to the fresh gasoline and then to permit the antioxidant to develop as peroxides are formed. In either case, it is necessary to develop only a small amount of the anti- 65 oxidant, which then serves to destroy catalytically the peroxides as formed thereafter.

Instead of depending on the peroxides formed in the gasoline as the oxidizing 70 agent, I may use other oxidizing materials. Thus, I may use any of the well known oxidizers described in the literature, but I prefer to use in such cases soluble organic oxidants, such as benzoyl peroxide, cyclo- 75 hexene peroxide, etc. The oxidizing agent may be dissolved in the gasoline either before or after the addition of the components of the antioxidant, and the production of the antioxidant quickly obtained. 80

The reaction between the components of the antioxidant and the oxidizer usually takes place smoothly at room temperature, but in some cases it may be desirable to warm the gasoline slightly, say around 85 100° F. to 200° F. If the gasoline is extremely volatile at the reaction temperature, then it is advantageous to reflux the vapors, or preferably to maintain on the oil a substantial superatmospheric pressure, 90 for example the pressure self-generated by confining the evolved vapors, to prevent boiling away of the lighter constituents.

The components capable of forming antioxidants that may be added to the gasoline comprise, preferably, two groups: (1) quinones, phenols and naphthols; and (2) aromatic amines, phenylenediamines and amino phenols. In practicing the invention, I select at least one compound from 100

each of the above groups and add a predetermined amount to the gasoline to be treated. It is to be understood, however, that the invention is not limited to the materials just mentioned but is equally applicable to all materials capable of oxidizing to an antioxidant and it is accordingly contemplated to include all such materials within the scope of the invention.

10 Many of the antioxidants produced in this way are coloring agents or dyes and therefore I may simultaneously develop in the gasoline a dye of suitable color, for example ranging from red to blue. Also, I 15 may add the components of the antioxidant to a gasoline which is already colored with dye, such as a red or blue gasoline, and not only inhibit oxidation of the gasoline, but also stabilize the color of the dye already 20 in the gasoline. Accordingly, I may select suitable components which will develop color similar to the dye already in the gasoline and thereby augment the color as required; thus, if the gasoline is colored with 25 a red dye, I may add components which will develop a red color and as the dye tends to fade, the color of the antioxidant will serve as an auxiliary coloring agent to maintain a constant shade.

30 As an example of one way of practicing the invention, I may add to a cracked gasoline 30 mg. of alpha-naphthol and 20 mg. of para-phenylenediamine per liter of the oil. If peroxides are present, or if they are 35 formed, they are reacted with the above compounds to form an indophenol, as will be indicated by a bluish color. It will be observed that in case the gasoline already contains a dye, the color will be gradually 40 augmented. Also, in case it is desired to hasten the reaction, which may sometimes be slow if dependent on the formation of peroxides, an organic peroxide such as benzoyl peroxide may be added. The resulting 45 gasoline is found to be substantially increased in resistance toward oxidation.

Instead of para-phenylene in the above example, I may use a substituted derivative, such as dimethyl or diethyl para-phenylenediamine, or I may substitute therefor an aminophenol, say ortho-aminophenol, or I may use instead of either of the foregoing an aromatic amine or a substituted amine, for example aniline or dimethyl aniline. 55 Also, I may replace the alpha-naphthol in the above example with hydroquinone or naphthaquinone.

Obviously many modifications and variations of the invention, as hereinbefore set forth, may be made without departing from the spirit and scope thereof, and therefore only such limitations should be imposed as are indicated in the appended claims.

What I claim is:

65 1. The method of treating cracked gaso-

line to increase the resistance thereof toward oxidation which comprises adding the components of an antioxidant to the gasoline and then developing the antioxidant in situ by reacting said components with an oxidizing agent. 70

2. The method according to claim 1 in which the oxidizing agent consists of an organic peroxide.

3. The method according to claim 1 in 75 which the oxidizing agent consists of peroxides formed by autoxidation of the gasoline.

4. The method of producing an antioxidant in cracked gasoline which comprises adding the components of an antioxidant to a gasoline containing preformed peroxides and then reacting said components with the peroxides to develop in situ the antioxidant. 80

5. The method of treating cracked gasoline which comprises adding to the gasoline 85 components capable of producing an indophenol and then developing the indophenol in situ by oxidation with peroxides formed by autoxidation of the gasoline.

6. The method according to claim 5 in 90 which the components comprise at least one compound selected from each of the two groups consisting of: (1) phenols, naphthols and quinones; and (2) aromatic amines, phenylenediamines and aminophenols. 95

7. A motor fuel comprising gasoline to which has been added the components of an antioxidant, said components including at least one compound selected from each of the two groups consisting of: (1) phenols, naphthols and quinones; and (2) aromatic amines, phenylenediamines and aminophenols. 100

8. A composition of matter comprising cracked gasoline which contains in solution 105 an antioxidant of the indophenol type developed in situ by the oxidation of the components of the antioxidant while dissolved in said gasoline.

9. The method of treating cracked gasoline which comprises adding to the gasoline at least one compound selected from each of the two groups consisting of: (1) para-phenylenediamine and its substituted derivatives; and (2) phenol and alpha-naphthol; 115 and then oxidizing said added components while in solution in said gasoline whereby there is formed in situ an antioxidant of the indophenol type.

10. A composition of matter comprising 120 cracked gasoline which contains in solution an antioxidant resulting from the oxidation in situ of at least one compound selected from each of the two groups consisting of: (1) para-phenylenediamine and its substituted derivatives; and (2) phenol and alpha-naphthol. 125

In witness whereof I have hereunto set my hand this 20th day of February, 1932.

LEO P. CHEBOTAR. 130